

B. E. STRONG & H. G. CLEMENGER.  
METHOD OF BLEACHING VENEERS.  
APPLICATION FILED MAR. 30, 1914.

1,128,073.

Patented Feb. 9, 1915.

3 SHEETS-SHEET 1.

Fig. 1



Fig. 2.



Fig. 3.



Witnesses  
Haslandberg  
Harold Forsberg

By *Berdette E. Strong*  
*and Harry G. Clemenger*  
*S. Arthur Baldwin.*  
Attorney

B. E. STRONG & H. G. CLEMENGER.  
METHOD OF BLEACHING VENEERS.  
APPLICATION FILED MAR. 30, 1914.

1,128,073.

Patented Feb. 9, 1915.

3 SHEETS—SHEET 2.



Inventors

Berdette E. Strong  
and Harry G. Clemenger  
By S. Arthur Baldwin.

Attorney

Witnesses  
H. A. Sandberg  
Harold Sandberg

B. E. STRONG & H. G. CLEMENGER.

METHOD OF BLEACHING VENEERS.

APPLICATION FILED MAR. 30, 1914.

1,128,073.

Patented Feb. 9, 1915.

3 SHEETS—SHEET 3.



Witnesses  
Harold Forsburg.  
Orslandberg.

Perdette E. Strong  
and Harry G. Clemenger  
By  
S. Arthur Baldwin, Attorney

# UNITED STATES PATENT OFFICE.

BERDETTE E. STRONG AND HARRY G. CLEMENCER, OF JAMESTOWN, NEW YORK.

## METHOD OF BLEACHING VENEERS.

1,128,073.

Specification of Letters Patent.

Patented Feb. 9, 1915.

Application filed March 30, 1914. Serial No. 828,204.

*To all whom it may concern:*

Be it known that we, BERDETTE E. STRONG, and HARRY G. CLEMENCER, citizens of the United States, residing at the city of Jamestown, in the county of Chautauqua and State of New York, have invented certain new and useful Improvements in Methods of Bleaching Veneers, of which the following, taken in connection with the accompanying 10 drawings, is a specification.

The invention relates to a process of bleaching veneer or thin boards; and the object of the improvement is, first, to provide a method of bleaching veneer in sheets 15 wherein a desired number of sheets are assembled or supported together so as to be simultaneously submerged and treated in a bleaching solution and held separated from one another by an interposed medium in 20 such a manner that the bleaching solution may come in contact with the entire surfaces of the veneer sheets allowing the operation to be economically carried out without injury to the sheets; and second, to provide a process in which the sheets are held 25 separated by open work textile or wire fabric such as textile net or webbing or coarse wire fabric which will not be affected by the chemicals in the bleaching solution to 30 thereby discolor or injure the veneer sheets and yet which will last for an indefinite period, thereby insuring great economy in the use of the process; and the invention consists in the novel combinations hereinafter 35 set forth and claimed.

In the drawings, Figure 1 is a side elevation of a separating screen or medium with fairly close mesh or weave; and Fig. 2 shows a similar separating screen or medium 40 with coarse mesh. Fig. 3 is a perspective view of a portion of the bleaching vat with the sheets of veneer separated by the screens, a single screen between each of the sheets of veneer, the sheets of veneer, the 45 screens and vat being shown in vertical section. Fig. 4 is a sectional view at line X X in Fig. 2, showing the preferred manner of constructing the separating screen with undulations in the strands of the coarse mesh 50 of the fabric. Fig. 5 is a plan view of a sheet of veneer to be bleached. Fig. 6 is an elevation of a plurality of boards or sheets of veneer separated by coarse cloth, netting or other flexible material. Fig. 7 is an elevation 55 of a plurality of sheets of veneer

separated by cloth or other porous flexible material with separating frames at spaced intervals to insure the firm holding of the sheets of veneer so that they will not warp out of line. Fig. 8 is a perspective view of 60 a portion of the bleaching vat with a plurality of sheets of veneer separated by coarse cloth, netting or other flexible material and pairs of separating frames or screens at spaced intervals and arranged 65 upon their edges in said vat, the screens, separating material, veneer and vat being shown in vertical section. Fig. 9 is a perspective sectional view of the bleaching vat with the thin boards or veneer suspended 70 from rods in the top of the vat with weights on their lower edges and placed alternately with sheets of coarse cloth, netting or other porous material which form a separating 75 medium between the sheets of veneer or boards. Fig. 10 is a sectional elevation of the bleaching vat lengthwise of the sheets of veneer and separating medium, showing the sheets of veneer suspended from a plurality of cross rods. Fig. 11 is an elevation 80 of one of the hooked clamps for supporting the veneer on the cross rods and attaching the weights on the lower edges of the sheets of veneer.

Like numerals of reference refer to corresponding parts in the several views.

The numeral 10 designates a bleaching vat which should be sufficiently large to hold the sheets of veneer or boards 14, which vary in size, and to hold sufficient of the 90 bleaching compound 13 to cover the veneer when placed in the vat 10.

The sheets of veneer 14 are usually cut from logs from four to twelve feet in length, and some sheets are the full length of the 95 log and the full cut around the periphery of the log, often attaining a width of four feet. The difficulty in firmly holding such a large sheet of thin veneer separate from other sheets within the bleaching liquid 100 without warping will be appreciated.

It is essential that the sheets of veneer or boards should not be permitted to contact with one another in the bleaching compound until the sap or native juices are entirely extracted. Should they contact with one another before the extraction of the sap they would badly discolor one another at each point of contact, since the chemical action of the bleaching compound upon the 110

wood before the extraction of the sap causes such a discoloration or spotting. The separating medium must at the same time permit the free access of the bleaching compound to the entire surface of the veneer or boards 14. After the extraction of the sap the contacting of the veneer or boards does not discolor the same.

There are different ways of supporting the veneer or thin boards and the separating medium therefor in the bleaching compound. The assembled boards or veneer with the separating medium placed therebetween may be bound in a bundle and rest upon edge on raised bars 11 on the bottom 12 of the vat 10, or they may be hung from cross bars 20 at the top of the vat 10 in which case they would need weights 24 at the lower edges to keep the thin boards firmly in line.

When the veneer or thin boards 14 are placed on edge on the bars 11 the separating medium or frames supporting the sheets of veneer should be sufficiently strong to firmly hold the sheets in line. Accordingly a separating frame or screen 15 is provided, having a substantially close woven mesh 16 for certain woods, or a coarse mesh 17 for others. The material used for the strands of the mesh 16 and 17 may be such that it will not discolor the boards or veneer 14 or affect the bleaching compound 13. Textile netting is preferred, though tinned woven wire will accomplish the purpose.

It is apparent that a solid flat surface would not permit the access of the bleaching compound to the sides of the boards or sheets of veneer 14, accordingly a porous medium is required. The strands of the mesh 16 and 17 are preferably made in undulating form, as shown in Fig. 4, so that the spaced undulations or points contact at regular intervals against the side of the veneer when placed along side the same, thereby holding the entire sheet of veneer or thin board firmly in line by pressing upon all parts of the same at spaced intervals.

To insure the absolute separation of sheets of delicate veneer, as for example bird's-eye maple, a strip of fabric 18, like coarse cloth, netting or other bendable material, may be wrapped about the sheets of veneer 14, being folded back and forth as the veneer is placed upon the same or laid alternately therewith so as to place a thickness of the material between the sides of two adjacent sheets.

It is apparent, however, that a series of thin sheets of veneer need additional support beside the cloth in order to stand on their edges. Accordingly, a single or a pair of screen frames 15 are inserted at spaced intervals between the separated sheets of veneer or bound therewith, and the whole mass is placed edgewise in the vat 10 upon the supporting bars 11 in the same manner that the heavier boards or veneers shown in

Fig. 3 are placed on edge, and the bleaching compound 13 is then flowed about the veneers by filling the vat or the bound sheets of veneer and separating medium may be submerged in the compound. The wood veneer has to be held beneath the surface of the bleaching compound, otherwise it would float and not stay submerged and thereby stop the bleaching process.

The alternate sheets of veneer and coarse cloth, netting or other porous material may be hung from rods 20 supported on the upper edge or near the upper edge of the vat in holes 19 or notches 26. The sheets of cloth 22 may be arranged with eyelets 21 and slipped onto the rods 20 or may be hung therefrom the same as the sheets of veneer 10. For long sheets of veneer a plurality of rods 20 should be provided and a small clamp 25 with a hook 23 attached thereto for hooking over the rods 20. The same clamp 25 is also used for clamping the lower edge of the veneer 10 and hanging a weight 24 thereon to hold the veneer in line. It is apparent that the sheets of cloth 22 could be supported from the rods 20, the same as the sheets of veneer 10, and that this arrangement holds the veneer in the bleaching compound.

It is obvious that it would not depart from our invention to lay the sheets of veneer or thin boards 14 flat upon their sides on the supporting bars 11 instead of supporting them on their edges on said bars or hanging them from the bars 20. It is found however that the bleaching compound 13 works up between the sheets of veneer with greater freedom when placed vertically in the vat 10, and that all parts of each board or sheet of veneer are thus more thoroughly and quickly approached by the bleaching compound.

We claim as new:—

1. The herein described method of bleaching veneer sheets consisting in assembling a plurality of veneer sheets and interposing a separating medium between said sheets of veneer to prevent their touching one another, and then submerging the same in a bleaching solution.

2. The herein described method of bleaching veneer sheets, consisting in assembling a plurality of veneer sheets and interposing a porous separating medium between said sheets of veneer to prevent their touching one another, and then submerging the same in a bleaching solution.

3. The herein described method of bleaching sheet veneer, consisting in assembling a number of sheets together with interposed layers of a textile fabric, and then submerging the assembled veneer and fabric in a bleaching solution.

4. The herein described method of bleaching veneer sheets, consisting in assembling

a plurality of sheets of veneer in bundle form with interposed layers of fabric netting, and then dipping the bundle in a bleaching solution.

5. The herein described method of bleaching veneer sheets, consisting in assembling a plurality of sheets of veneer and interposing a separating medium between said sheets comprising intercrossed threads or

wires, and submerging the same in a bleaching solution.

In testimony whereof we have affixed our signatures in the presence of two witnesses.

BERDETTE E. STRONG.  
HARRY G. CLEMENGER.

Witnesses:

H. A. SANDBERG,  
HAROLD FORSBERG.